

Oct. 31, 1933.

W. L. WRIGHT

1,933,466

PAPER AND OTHER FIBROUS SHEET MATERIAL HOOD CAP

Filed Nov. 30, 1925

Fig. 1.



Fig. 2.



Fig. 3.



Fig. 4.



Inventor  
by Wilbur L. Wright  
by Hubert E. Peck  
Attorney.

## UNITED STATES PATENT OFFICE

1,933,466

PAPER AND OTHER FIBROUS SHEET  
MATERIAL HOOD CAPWilbur L. Wright, Fulton, N. Y., assignor to  
Oswego Falls Corporation, Fulton, N. Y., a  
corporation of New YorkApplication November 30, 1925  
Serial No. 72,318

11 Claims. (Cl. 215—38)

This invention relates to hood caps, particularly to binder-carrying hood caps; and an object of the invention is to provide a fibrous or other paper like hood cap for bottles and other containers, provided with a binder composition that includes sulphur as an ingredient.

With this and other objects in view, my invention consists in certain novel features, and in a novel material and a novel article, as more fully and particularly set forth and specified hereinafter.

Referring to the accompanying drawing forming a part hereof:

Fig. 1 is a side elevation of the mouth portion 15 of a container, such as a so-called milk bottle, covered by a hood cap or cover, more or less diagrammatically illustrated as including or embodying my invention.

Fig. 2 shows the structure of Fig. 1, in vertical section.

Fig. 3 is a plan view of a sheet of paper or other fibrous material embodying my invention.

Fig. 4 shows a sheet material hood cap in accordance with or embodying my invention, in form for application to a container to cover and protect the mouth thereof.

In the drawing, I show the head or mouth portion of a glass milk bottle (to represent any suitable container) having exterior annular enlargement 30 or vertically rounded rim 1, that radially contracts inwardly and downwardly to the neck 2, of the container to form annular downwardly facing shoulder or contraction 3.

I propose to retain the skirt of the hood cap in rigid contracted form under the enlarged bottle head and tightly surrounding and fitting and preferably sealing against the bottle neck by the use of sheet material impregnated with or carrying a strong hard high-melting point quickly setting binder composition, preferably light in color, that embodies sulphur and one or more additional modifying ingredients, whether such impregnated sheet material constitutes the annular lower or securing portion of the hood cap skirt, or is formed by an extra securing ring of such impregnated sheet paper or like material surrounding the skirt for holding the same tightly contracted to the bottle neck against leakage and against accidental release.

When this impregnated or coated sheet material hood cap disk is rendered soft or pliable by the necessary heat, it can be worked or molded by suitable mechanism to contract the cover skirt tightly to and around the bottle neck. Such mechanism will then maintain the soft sheet

material in such form, until the impregnated material sets to rigid cap securing form by cooling as it does quickly within a few seconds. The set impregnated material is then of sufficient stiffness and tensile strength to hold the hood cover sealed on the bottle mouth against accidental removal and looseness. However, by the exercise of sufficient strength, the cover can be stripped from the bottle mouth when necessary.

In Figs. 1, 2 and 4 of the drawing I show a sheet 65 paper material hood cover or cap 4 to cover the mouth portion of a bottle or other container, and formed with an annular depending skirt 5 of sufficient length to permit contraction thereof below the bottle rim 1 to surround and closely fit the 70 bottle neck 2 under the exterior enlargement of the bottle head, with the ends in view of locking the cap on the bottle mouth and sealing the bottle mouth against passage of liquid to the interior thereof. The portion 6, of the cover or cap skirt 75 that is contracted below the bottle rim, to lock or secure the cap, by the formation of said portion into gathers, ridges, corrugations, puckers, overlapping pleats or crimps 6a, which I call the securing portion of the cover or cap skirt. In the 80 example shown, it is this annular portion 6 of the cap or cover skirt that possesses the hereinbefore mentioned characteristics by reason of the impregnating binder carried thereby, although I do not wish to so limit my invention as the cap or 85 cover can in whole or in part embody the binder.

The caps or covers are usually produced and shipped in the tapered or flaring form shown by Fig. 4, so as to be readily applicable to the bottle mouths.

Dies are usually employed to draw the thin or single ply sheet paper material from disks such as shown by Fig. 3, into the form shown by Fig. 4, although, if desirable, the bottlers can be supplied with the flat disks of Fig. 3, for use in machines that will properly shape such disks and finish them on the bottle mouths in the form of hoods as in Fig. 1.

Whether the sheet material is supplied the bottler in the form of Fig. 3 or in the form of Fig. 4, such sheet material throughout, or only at the securing portions 6 thereof embodies the binder as indicated by the dotted field, and is heated to the necessary temperature to render said binder carrying securing portion pliable, soft, or moldable, immediately before application to the bottle, or by the molding head that molds the same to form, snugly fitting the bottle neck and under the bottle head enlargement.

The hood cap disks, preferably in the form of 110

Fig. 4, are subjected, in any suitable manner or by any suitable means, to the binder in hot liquid form so that, at least the annular securing portions of the cap skirts, become impregnated with the hot liquid binder and on cooling set in rigid form.

This composition is produced by reducing the sulphur and a hard quick setting wax or waxes to liquid form by heat and mixing the ingredients.

10 In producing my sulphur-wax binder composition, I usually mix the molten wax with a surplus quantity or over-supply of molten sulphur, so that the melted wax will take up as much sulphur as possible, i. e. the melted wax will take up 15 sulphur until saturated, and when agitation of the mixture ceases, the surplus sulphur settles or is precipitated, and the sulphur-wax composition can be drawn off.

As the wax ingredient, I prefer to employ 20 carnauba wax, although Montan wax, candelilla wax, shellac wax, or "Smith & Nichols" vegetable wax, or other hard high-melting point quick setting waxes, can be employed, with or without the addition of other ingredients in small proportion 25 to add strength, or to prevent bottle fouling in such sulphur and wax composition that would otherwise objectionably foul glass.

Candelilla, carnauba, and "Smith & Nichols", are vegetable waxes of commerce and are thus 30 known in the wax trade. Montan wax is a mineral wax of commerce, and is known to the wax trade. Shellac wax is an insect product.

Montan is imported from Europe and is believed to be derived from thuringian lignite. I employ 35 refined or bleached Montan wax, which in color ranges from white to yellow, and has a melting point from about 160° to 170° F., is a solid at climatic or atmospheric temperatures, has a characteristic aromatic odor, and is approximately 40 insoluble in cold alcohol.

Smith & Nichols vegetable wax is produced in a foreign country, and its importation into this country is apparently controlled by Smith & Nichols of New York, N. Y., as it is known commercially and named in price lists as "Smith & Nichols" or "S. & N." vegetable wax. This product is dark brown in color, hard, with a slight strawlike odor when cold and a characteristic sweet odor when heated, with a melting point of 50 about 160° to 165° F.

Ordinary commercial sulphur in any of its various forms might be employed, but I preferably use lump sulphur. The wax and sulphur are preferably separately reduced to liquid form and are 55 drawn from their respective kettles or receptacles into a common kettle or receptacle wherein the two liquids are mixed and kept at a temperature of approximately from 235° to 300° F. between which temperatures the ingredients seem to combine or mix with the resulting binder composition containing approximately between one and two percent sulphur.

The impregnated paper material quickly cools 60 at atmospheric or climatic temperatures, and sets to a condition of stiff rigidity. The rigid stiff impregnated paper material becomes soft and moldable at a temperature of say about 210° F. more or less where the composition is composed of carnauba wax and sulphur, and is thus heated for 70 contracting around the bottle neck by suitable mechanism.

Many of the hard unrefined hard quick setting waxes of commerce, suitable for use as hood cap 75 binders, as found on the market, are dark in color

and dirty and objectionable in appearance for hood cap binder purposes.

I have discovered that these waxes are lightened in color by the sulphur treatment, and that the resulting composition is of a lighter clearer color 80 than the original wax, and is also otherwise rendered more desirable for hood cap binder purposes by the presence of the small sulphur percentage or proportion, in that the composition is somewhat harder and denser, and has greater water 85 resistant qualities than the original wax, and is cheaper in cost than the original wax because of the very low cost of sulphur. The melting point of the composition seems to vary but slightly from that of the wax ingredient in its original condition, but the composition is otherwise more desirable for hood cap binder purposes than the original wax ingredient.

A dark mineral wax, such as Montan wax, will 90 take up the small sulphur percentage to form the sulphur-wax binder composition but such composition is but slightly cleared and lighter in color than the original Montan wax, but where hard waxes of vegetable and insect origin are 95 mixed with sulphur the resulting composition is 100 decidedly lightened and clear in color, and this desirable result is also gained where a small proportion of a water-resistant strong yet sticky substance, such as rosin, say about five percent, is added to the composition to increase the 105 strength and water resistant qualities thereof without rendering the composition so adhesive as to foul glass bottles or form deposits thereon that cannot be easily rubbed or stripped therefrom. The degree of adhesiveness of such compositions 110 can be regulated or predetermined by the percentage or proportion of the rosin or like ingredient, to gain, where desired, a slight adhesion between the binder carrying skirt of the hood cap and the glass bottle surface for sealing purposes 115 without leaving an objectionable bottle fouling deposit on the glass when the cap skirt is stripped therefrom. Also where a wax, such as candelilla wax, is employed as the wax ingredient in the sulphur-wax composition, a small percentage of 120 some grease-like substance, such as paraffine, can be added to prevent the resulting binder composition from being objectionably adhesive on glass surfaces or from leaving a glass fouling deposit 125 on bottles. The adhesive qualities of such a composition can be regulated and predetermined by varying the proportion of the grease-like ingredient but the percentage of such ingredient must be small as the strength and hardness of such binder composition is thereby reduced and its melting 130 point thereby lowered.

By adding sufficient wax to the sulphur, and then applying the hot liquid binder composition to the sheet material, I provide impregnated hood cap securing sheet material that possesses great 135 tensile strength and rigidity, is insoluble and non-absorbent for my purposes, is of a desirable color, is not objectionably brittle, is tasteless, odorless, light in color, non-poisonous, does not attract insects or vermin, with the exceptions mentioned 140 does not stick to glass or metal or foul or adhere to the contracting crimping heads or tools when hot, sets or hardens quickly, is easily contracted and pressed on the bottle necks when hot, and will not mold or mildew.

While the impregnated sheet material will with great strength adhere to itself as when pleats or tucks therein or walls or portions thereof are pressed together.

Fig. 2 of the drawing is not intended to indicate 150

- or give the impression that the impregnated or securing portion 6 is stuck or adhered to the glass bottle neck as such is not the fact, nor is said figure of the drawing intended to indicate a substantial or really visible surface coating of sulphur or sulphur and wax on the paper material but is intended to indicate rigidly adhering overlapping folds, pleats, or creases of the impregnated material.
- 10 For use in connection with hood caps or covers on glass bottles of food products, it is desirable that the impregnated sheet material be non-glass fouling both when hot and cold, and possess the quality of stripping or peeling from glass surfaces, and this is a peculiar characteristic of carnauba and certain other of the waxes and compositions mentioned.
- The binder composition is saturated with and modified by the sulphur dispersed therethrough and alloyed or blended with the other ingredient or ingredients of the composition which act to retard, decrease or modify the crystallization of the sulphur after fusing.
- The instant application is a continuation in part 25 of my patent application Serial No. 722,353, filed June 25, 1924, for paper and other fibrous sheet material.
- What I claim is:
1. A sheet fibrous material hood cap carrying a quick-setting hard water-resistant plastic binder composition that embodies a small percent of sulphur.
  2. A sheet paper-like hood cap carrying a hard quick-setting binder embodying wax saturated with sulphur, the binder being of a lighter color than the wax in its original condition.
  3. A paper material hood cap carrying a binder composition embodying a hard wax and a small percent of sulphur, the composition being lighter in color than the wax before being mixed with the sulphur.
  4. A paper material hood cap carrying a binder composition of carnauba wax and sulphur.
- 45
- 50
- 55
- 60
- 65
- 70
- 75
- 80
- 85
- 90
- 95
- 100
- 105
- 110
- 115
- 120
- 125
- 130
- 135
- 140
- 145
- 150
5. A hood cap composed of a single ply disk of sheet paper carrying at its skirt portion a binder composition of a hard quick setting wax-like plastic embodying and lightened in color by sulphur.
6. A bottle sealing paper material hood cap at least the peripheral portion of which carries a binder composition of matter comprising sulphur and a substance capable of retarding the crystallization of sulphur.
7. A hood cap composed of sheet paper and a quick setting hard water resistant binder composition embodying a plastic saturated with sulphur.
8. A hood cap of fibrous sheet-form material, carrying a quick setting water resistant plastic binder saturated with sulphur and which is a hard solid when cold.
9. A hood cap of fibrous sheet form material, carrying a quick-setting water resistant plastic binder which is a hard solid when cold, which binder contains a proportion of sulphur and a substance blended therewith and which remains blended therewith on heating and cooling.
10. A milk bottle sealing cap carrying in a sealing position, a sealing composition comprising sulphur and an agent which acts to prevent prompt crystallization of the sulphur and also acts to somewhat change the melting point of the sulphur.
11. A bottle cap of paper the lower edge portion of which is adapted to be crimped and molded over the mouth of the bottle, said crimped portion carrying intimately bonded thereto, a binder mixture comprising essentially sulphur and a substance which will modify and decrease the crystallizing properties of sulphur, said binding mixture stripping readily from the bottle glass surface on removal of the cap therefrom.
- WILBUR L. WRIGHT.